

Patented Nov. 19, 1940

2,222,285

# UNITED STATES PATENT OFFICE

2,222,285

## AGENTS FOR AFTERTREATING DYEINGS OF INSOLUBLE AZO DYESTUFFS

Hans Ellner, Stuttgart, Germany, assignor, by  
mesne assignments, to General Aniline & Film  
Corporation, New York, N. Y., a corporation of  
Delaware

No Drawing. Application April 7, 1938, Serial  
No. 200,678. In Germany April 27, 1937

8 Claims. (Cl. 8—74)

The present invention relates to agents for  
aftertreating dyeings of insoluble azo dyestuffs  
produced by coupling on the fiber, and a process  
of improving the fastness to rubbing of dyeings  
produced by means of insoluble azo dyestuffs.

Dyeings produced by means of insoluble azo  
dyestuffs, by coupling on the textile fiber, are  
generally subjected to an aftertreatment at boil-  
ing temperature, in most cases with soap or with  
10 soap and sodium carbonate. By this after-  
treatment, it is intended to fix the shade, to im-  
prove the fastness, especially the fastness to  
light, and to enhance the fastness to rubbing. In  
many cases it is, however, not possible, even  
when most carefully working, to obtain, with re-  
spect to the fastness to rubbing, results which  
are sufficiently good for all purposes.

I have found that the fastness to rubbing of  
dyeings produced by means of insoluble azo dye-  
stuffs by coupling on the textile fiber may be im-  
proved to a considerable degree by using for the  
aftertreatment at the boil liquors containing,  
besides the washing agent, inorganic or organic  
salts which react with salts or hydroxides of the  
alkaline-earth metals to form water-soluble  
compounds. The fastness to rubbing is, in many  
cases, further improved and the beauty of the  
shade is enhanced if an agent yielding oxygen is,  
furthermore, added to the liquor.

Washing agents suitable for use in the pres-  
ent process are synthetic organic surface active  
detergents such as for instance: alkali soaps  
from saturated or unsaturated fatty acids, fatty  
alcohol sulfonates, condensation products from  
fatty acids and the halides thereof with aliphatic  
and aromatic amines and substitution products,  
and sulfonation products of such compounds,  
condensation products from ethylene oxide with  
aliphatic and mixed aliphatic-aromatic alcohols  
and phenols, and other wetting and dispersing  
agents.

Suitable inorganic and organic salts which re-  
act with salts, oxides or hydroxides of the alkali-  
ne-earth metals to form water-soluble com-  
pounds are, for instance: pyrophosphates, meta-  
phosphates, alkali salts of amino acids contain-  
ing a tertiary nitrogen atom and more than one  
carboxylic acid group for each nitrogen atom,  
such as nitrilo-triacetic acid, ethylene-bis-imido-  
diacetic acid.

As agents yielding oxygen there may be named  
as examples: perborates and persulfates, stabil-  
ization products from hydrogen peroxide with  
phosphates. These agents are used in propor-  
tions which are only fractions of those usually  
applied for oxygen bleaching.

The knowledge of this fact is very valuable  
and it could not be foreseen, especially since  
other salts than the inorganic and organic salts  
claimed, such as do not react with the alkaline-

earth salts to form water-soluble compounds, for  
instance sodium carbonate, trisodium phosphate  
and the like have not the above-described action  
and since larger amounts of agents yielding oxy-  
gen destroy the dyestuff. The favorable action  
of the mixture of the washing agent and salts  
forming soluble salts with the alkaline-earth  
metals and of agents yielding oxygen occurs al-  
ways, it being immaterial whether the preceding  
dyeing process has been performed in soft or 10  
hard water.

The new process is especially valuable in the  
dyeing of laps, cross wound bobbins, warp beams  
and the like and avoids the use of fat-containing  
15 washing agents.

The following examples serve to illustrate the  
invention, but they are not intended to limit it  
thereto:

(1) A dyeing, produced in known manner by  
coupling on the fiber 5 grams of 1-(2',3'-hydroxy-  
naphthoylamino)-2-methyl-4-methoxybenzene  
per liter and the diazo compound from 2 grams  
of 2-methyl-4-chloro-1-aniline per liter, the ratio  
of the goods to the liquor being 1:20, is well  
rinsed after dyeing and introduced into an after-  
treating bath having a temperature of 50° C. and  
containing per liter of softened water 0.3 gram  
of isoctylphenyl-polyglycol ether with 10 mols of  
ethylene oxide per molecule and 0.6 gram of the  
sodium salt of nitrilo-acetic acid. The whole  
is heated to boiling temperature, the material is  
treated, at this temperature, for about half an  
hour, rinsed hot and cold and dried; a red dyeing  
of very good fastness to rubbing is obtained.

If there is used, instead of 0.6 gram of the  
sodium salt of nitrilo-triacetic acid, the tetraso-  
dium salt of ethylene-bis-imidodiacetic acid,  
there are, likewise, obtained dyeings having a  
very good fastness to rubbing.

(2) A dyeing, produced in known manner by  
coupling on the fiber 4 grams of 1-(2',3'-hy-  
droxynaphthoylamino)-4-anisol per liter and the  
diazo compound from 1.75 grams of 1-amino-2-  
methoxy-4-nitrobenzene per liter, the ratio of  
the goods to the liquor being 1:20, is well rinsed  
after dyeing and introduced into an aftertreat-  
ing bath having a temperature of about 50° C.  
and containing per liter 0.3 gram of isoctyl-  
phenyl-polyglycol ether with 10 mols of ethylene  
oxide per molecule, 1 gram of sodium pyrophos-  
phate and 0.5 gram of sodium perborate. The  
whole is heated to boiling temperature, the ma-  
terial is treated, for about half an hour, at this  
temperature, rinsed hot and cold and dried; a  
beautiful bordeaux dyeing having a very good  
fastness to rubbing is obtained.

(3) A dyeing, produced in known manner by  
coupling on the fiber 3 grams of 1-(2',3'-hy-  
droxynaphthoylamino)-4-chloro-2-methylben-  
zene per liter and the diazo compound from 2

grams of 2-methyl-4-chloro-1-aniline hydrochloride, the proportion of the goods to the liquor being 1:20, is well rinsed after dyeing and introduced into an aftertreating bath having a 5 temperature of 40° C.-50° C. and containing per liter 0.3 gram of isoctyl-phenol-polyglycol ether with 10 mols of ethylene oxide in the molecule, 0.3 gram of the sodium salt of nitrilo-triacetic acid and 0.5 gram of sodium perborate. The 10 whole is heated to boiling temperature, the material is further treated, for about half an hour rinsed hot and cold and dried. A beautiful red dyeing of very good fastness to rubbing is obtained.

15 (4) A dyeing, produced in known manner by coupling on the fiber 4 grams of 1-(2',3'-hydroxynaphthoyl)-amino-2,4-dimethoxy-5-chlorobenzene per liter and the diazo compound from 2.8 grams of 1-amino-2-methoxy-5-sulfo-20 diethylaminobenzene per liter the ratio of the liquor to the goods being 20:1 is well rinsed and treated, at about 50° C., with a bath containing per liter 0.3 gram of isoctyl-phenol-polyglycol ether with 10 mols of ethylene oxide in 25 the molecule, 0.3 gram of the tetrasodium salt of ethylene-bis-imido-acetic acid and 0.5 gram of sodium perborate. The bath is heated to boiling temperature, the material is further treated for half an hour, then rinsed hot and 30 cold and dried. A red dyeing of a surprisingly good fastness to rubbing is obtained.

(5) A dyeing prepared according to the indications made in Example 3 is well rinsed and introduced, at about 50° C., into a bath containing per liter 3 cc. of a lauric alcohol sulfonate 35 containing 27% of fat, 1 gram of sodium pyrophosphate and 0.5 gram of sodium perborate. The bath is heated to boiling temperature, the material is further treated for half an hour, rinsed hot and cold and dried. The red dyeing thus obtained displays a very good fastness to 40 rubbing.

(6) A dyeing obtained in the manner indicated in Example 1 is well rinsed and introduced, at 50° C., into a bath containing per liter 45 3 grams of Marseilles soap, 0.5 gram of sodium pyrophosphate and 0.5 gram of sodium perborate. The bath is heated to boiling and the material is further treated for about half an hour, then rinsed hot and cold and dried.

The bordeaux dyeing thus obtained has a very good fastness to rubbing.

(7) A dyeing obtained by coupling on the fiber 5 grams of 1-(2',3'-hydroxynaphthoyl)-amino-2-methyl-4-methoxybenzene per liter and the diazo compound from 2 grams of 1-amino-2-methyl-4-chlorobenzene hydrochloride per liter 55 is well rinsed and, at about 40° C.-50° C., introduced into a bath containing per liter about 0.5 gram of oleylmethyl-taurine, 0.5 gram of sodium perborate and 1 gram of sodium pyrophosphate. The bath is heated to boiling, the material is treated, for half an hour, at this temperature, then rinsed hot and cold and dried. The red dyeing obtained has a very good fastness to rubbing.

(8) A dyeing obtained according to the indications of Example 2 is rinsed and introduced, at about 50° C., into a bath containing per liter 60 0.4 gram of oleyl alcohol, oxethylated with 30 mols of ethylene oxide, 0.5 gram of sodium

pyrophosphate and 0.5 gram of sodium perborate. The bath is heated to the boil, the material is treated, for half an hour, at boiling temperature, then rinsed hot and cold and dried. The red dyeing obtained has a very good fastness to rubbing.

I claim:

1. A process of improving the fastness to rubbing of dyeings produced by means of insoluble azo dyestuffs, by coupling on the fiber, which consists in aftertreating the dyeings at boiling temperature with a liquor containing a synthetic organic surface active detergent and a metal salt which reacts with salts, hydroxides and oxides of the alkaline-earth metals to form water-soluble compounds.

2. The process as defined in claim 1, wherein said metal salt is a metaphosphate.

3. A process of improving the fastness to rubbing of dyeings produced by means of insoluble azo dyestuffs, by coupling on the fiber, which consists in aftertreating the dyeings at boiling temperature with a liquor containing a synthetic organic surface active detergent and a metal salt which reacts with salts, hydroxides, and oxides of the alkaline-earth metals to form water-soluble compounds and a small amount of an agent yielding oxygen selected from the group consisting of perborates, persulfates and stabilization products from hydrogen peroxide 30 and phosphates.

4. The process as defined in claim 3, wherein the metal salt is a metaphosphate.

5. A process of improving the fastness to rubbing of dyeings produced by means of insoluble azo dyestuffs, by coupling on the fiber, which consists in aftertreating the dyeings at boiling temperature with a liquor containing a synthetic organic surface active detergent and a pyrophosphate which reacts with salts, hydroxides and oxides of the alkaline-earth metals to form water-soluble compounds.

6. A process of improving the fastness to rubbing of dyeings produced by means of insoluble azo dyestuffs, by coupling on the fiber, which consists in aftertreating the dyeings at boiling temperature with a liquor containing a synthetic organic surface active detergent, a pyrophosphate which reacts with salts, hydroxides and oxides of the alkaline-earth metals to form water-soluble compounds and a small amount of an agent yielding oxygen selected from the group consisting of perborates, persulfates and stabilization products from hydrogen peroxide and phosphates.

7. A process of improving the fastness to rubbing of dyeings produced by means of insoluble azo dyestuffs, by coupling on the fiber, which consists in aftertreating the dyeings at boiling temperature with a liquor containing a synthetic organic surface active detergent and sodium pyrophosphate.

8. A process of improving the fastness to rubbing of dyeings produced by means of insoluble azo dyestuffs, by coupling on the fiber, which consists in aftertreating the dyeings at boiling temperature with a liquor containing a synthetic organic surface active detergent, sodium pyrophosphate and a small amount of sodium perborate.